

# UNITED STATES PATENT OFFICE.

HEINRICH KRETZER, OF WALLERSHEIM, NEAR COBLENZ, AND AUGUST CAPPEL, OF COBLENZ, GERMANY; SAID CAPPEL ASSIGNEE TO SAID KRETZER.

## PROCESS OF PRODUCING WELL-CLOUDED ENAMELS OR GLAZES BY MEANS OF SUBSTITUTES FOR STANNIC OXID.

1,239,112.

Specification of Letters Patent. Patented Sept. 4, 1917.

No Drawing.

Application filed September 9, 1914. Serial No. 860,883.

To all whom it may concern:

Be it known that we, HEINRICH KRETZER, doctor of chemistry, residing at Wallersheim, near Coblenz, and AUGUST CAPPEL, chemical engineer, residing at Coblenz, Germany, have invented certain new and useful Improvements in Processes of Producing Well-Clouded Enamels or Glazes by Means of Substitutes for Stannic Oxid, of 10 which the following is a specification.

As it is known, in modern enameling practice stannic oxid as well as the other specifying substances proposed in substitution are used in such a way that they are 15 added to the comminuted enamel proper when being ground in the wet-mill and that this mixture is subjected to the wet grinding operation until the enamel has been very finely ground—a condition necessary to laying-on the enamel. This wet 20 grinding operation generally continues for from five to ten hours.

If treated in this way most of the opacifiers other than stannic oxid, employed in 25 the manner described above and in quantities corresponding to the amount of stannic oxid commonly used, yield clouding effects totally insufficient. However, if used in larger 30 quantities they will produce injurious secondary phenomena or the process will become so expensive that an advantage worth mentioning will not arise over the use of stannic oxid.

Up to now it was generally believed that 35 this deficiency of opacifying power was due to the nature of the products themselves. Therefore, various proposals were made for removing this drawback by slightly modifying their chemical composition, however 40 without any remarkable success. Applicants' experiments with these substitute opacifiers proved that the intensity of the clouding or opacifying effect of any of the substances mentioned is by no means the 45 same with different enamels, but that it may vary within wide bounds. Moreover applicants have stated that the same clouding agent used in the manner described above may produce different opacities with the same enamel.

Now applicants have found that most of the enamels when being subjected to the wet grinding operation together with the opacifying agents have a decided tendency

to affect these substances and to transform 55 them into soluble forms (for instance by hydration, dispersion, formation of colloids, etc.). Contrary to stannic oxid which is not or only very slightly affected by the wet-milling process, these agents will lose 60 their clouding or covering power in the same measure as their alteration by the wet-milling process, that is to say, to the extent that the formation of soluble or instable 65 colloidal, etc., proceeds.

On the other side it has been found that the opacifying power of these substitute substances will not be diminished if all injurious influences during the wet milling process are removed. This may be effected 70 by avoiding or at least reducing the duration of the wet milling operation after having introduced the clouding agents in question or by adding such substances to the 75 enamel paste which in the wet milling operation will impede a colloidal transformation of the opacifying substance. As already mentioned stannic oxid does not suffer such injurious alterations, at least not in the measure as those substitute opacifiers which 80 contain zirconium, titanium, silicon, aluminum, zinc, alkaline metals, earth alkaline or earth metals or compounds of same. However, according to the invention, which is 85 the subject of the application, it is possible to obtain uniform and quite satisfying enamels with the substitute clouding agents mentioned.

In practice, this result is attained by failing to subject the opacifiers mentioned, as 90 it was the custom up to now, to the wet milling process during the same time as the enamel proper, but by adding same only after the enamel proper has undergone the wet milling process for the greatest part, 95 that is to say after the enamel has already got a fine and pasty condition.

The same result, although in a smaller measure is accomplished by introducing into the mill at the same time with the opacifying agents such substances which counteract to a transformation of the opacifiers into the colloidal or sol state, such as electrolytes (for instance chlorid of ammonium, sulfate or chlorid of magnesium, sulfate of sodium, etc.), as well as flocculating or precipitating collicids or similarly acting substances. From this point of view it ap-

pears also disadvantageous to let the finished milled enamel paste to settle any longer time as it has been proposed.

Finally it is to be remarked that antimonic products, for instance oxid of antimony, metaantimoniate of sodium, etc., act in a manner similar to stannic oxid regarding their being not altered in the wet mill. However, as it is known, antimonic compounds when used for enamel clouding purposes show the drawback that the enamel paste becomes slimy and is only with great difficulty to be laid on. For this reason heretofore only small quantities of antimonic opacifiers (4 to 5 per cent.) could be added to the enamel paste. We have found that the quantity of such antimonic opacifiers could be increased (twice, or more) and added to the enamels proper without the mentioned injuries being observed, if it is omitted to have these opaquing substances undergo the whole wet-milling operation together with the enamel proper, or if such substances as will counteract the formation of sols be added to the mass in the mill.

We claim as our invention:—

1. In the manufacture of white clouded enamels or glazes by means of opacifiers other than stannic oxid, the improvement which consists in adding the opacifying agents to the enamel proper when being

ground in the wet mill only after the milling process has been accomplished for the greater part.

2. In the manufacture of white clouded 35 enamels or glazes by means of opacifiers other than stannic oxid, the improvement which consists in adding to the enamel proper when being ground in the wet mill, the opacifying agents together with such 40 substances as will counteract a transformation of the opacifiers into colloidal forms.

3. In the manufacture of white clouded 45 enamels or glazes by means of opacifiers other than stannic oxid, the improvement which consists in adding to the enamel proper when being ground in the wet mill, the opacifying agents together with substances acting as electrolytes.

4. In the manufacture of white clouded 50 enamels or glazes by means of opacifiers other than stannic oxid, the improvement which consists in adding to the enamel proper when being ground in the wet mill, the opacifying agents together with substances acting as precipitating colloid.

HEINRICH KRETZER.  
AUGUST CAPPEL.

Witnesses:

A. H. SCHRODER,  
F. N. SEELEY.